# EUROPEAN PATENT SPECIFICATION

(11) **EP 1 937 884 B1**
(45) Date of publication and mention of the grant of the patent: **01.01.2014**
(21) Application number: 06793590.8
(22) Date of filing: 18.09.2006
(51) Int. Cl.: D04H 1/42, B22F 1/00

(54) **COATED POROUS METAL MEDIUM**
BESCHICHTETES PORÖSES METALLMEDIUM
SUPPORT MÉTALLIQUE POREUX REVÊTU

(30) Priority: 11.10.2005 EP 05109411
(43) Date of publication of application: 02.07.2008
(73) Proprietor: NV Bekaert SA, 8550 Zwevegem (BE)
(72) Inventor: GROENEN, Roland, B-9667 Horebeke (BE); VAN HEGE, Kris, B-9000 Gent (BE)
(86) International application number: PCT/EP2006/066449
(87) International publication number: WO 2007/042373

(56) References cited:
- EP-A- 1 205 602
- WO-A-99/56899
- GB-A- 2 394 428
- US-A- 4 270 936
- US-B1- 6 410 160

## Description

### Field of the invention.

The invention relates to a coated porous metal medium and to the use of such a coated medium as filter medium.

The invention further relates to a method of manufacturing a coated medium.

### Background of the invention.

Porous metal media comprising sintered metal fibers and/or sintered metal powder are well known in the art. They are for example used as filter media.

The in-depth coating of a porous metal medium may offer the medium many attractive properties such as corrosion resistance, chemical resistance, high temperature resistance, ...
However, it is hard to obtain a uniform and conformal coating throughout the thickness of the medium.
Many coating techniques have been tested without success. Most coating techniques do not allow to obtain a uniform and conformal coating throughout the thickness of the medium, for example because the outer pores of the medium are sealed before the interior can be coated.

By means of activated chemical vapour deposition such as hot filament the in-depth coating of a porous medium is not satisfactory.
In hot filament chemical vapour deposition for example, the process is generally so reactive that the precursor will react and will be deposited at the outer surface of the porous medium so that the interior of the medium will not be coated.
The in-depth coating of a porous metal medium by thermal CVD is a complex process and does not allow to coat the medium in-depth with a conformal coating layer that has a uniform composition and a constant coating thickness over the thickness of the medium.

### Summary of the invention.

It is an object of the present invention to provide a coated porous metal medium avoiding the problems of the prior art.

It is another object of the present invention to provide a coated porous metal medium whereby the whole free area surface S is coated.

It is a further object of the invention to provide a coated porous metal medium whereby the coating is conformal and uniform over the whole free area surface.

It is a further object of the present invention to provide a coated porous metal medium whereby the whole free area surface S of the medium is coated with a closed coating having a minimal thickness.

According to a first aspect of the present invention a coated porous medium comprising metal particles is provided.
The metal particles of the medium define a free area surface S, i.e. the total surface of the medium that is in contact or may have contact with air or another gas or that is in contact with the fluid to be filtered in case the medium is used for filtration.
The free area surface S includes thus not only the free area surface S at the outer surface of the medium, but also the free area surface S in the pores of the medium.
According to the present invention, the free area surface S of the metal surface is substantially completely coated with a coating layer. The coating layer is substantially conformal over the whole free area surface S; the coating layer is substantially uniform in composition over the whole free area surface S and has substantially the same thickness over the whole free area surface.

### Porous metal medium

The metal particles of the porous metal medium comprise preferably steel such as stainless steel. Preferred alloys comprise 316 L, FeCrAlloy^{®}, Alloy HR or Aluchrome^{®}.

The metal particles of the porous metal medium preferably comprise metal powder or metal fibers or a combination of metal powder and metal fibers.

The metal fibers have preferably a diameter ranging between 1 µm and 100 µm. More preferably, the diameter of the metal fibers is between 1 and 35 µm, for example 2 µm, 4 µm, 8 µm or 12 µm.
The metal fibers may be obtained by any technique known in the art. They are for example obtained by bundle drawing or shaving.

The porous metal medium may comprise a woven or a non-woven porous metal medium.

In a preferred embodiment the porous metal medium comprises a non-woven porous metal medium comprising sintered metal fibers.

In an alternative embodiment the porous metal medium comprises sintered metal powder.

In a further embodiment the porous metal medium comprises a combination of metal fibers and metal powder particles which have been sintered.

### Coating layer

The coating layer is preferably applied by atomic layer deposition (ALD).
ALD is a coating technique based on Chemical Vapor Deposition (CVD). In ALD a coating is applied by alternating exposures of the surface of two or more chemical reactants.
The ALD technique offers many advantages. ALD allows for example to obtain uniform, ultra thin coatings. Furthermore, the thickness of the coating can be precisely controlled on the atomic scale.

When ALD is used to apply a coating on a porous metal medium according to the present invention, a coated porous metal medium having unique characteristics is obtained.

First of all, as ALD allows to infiltrate into the pores of a complex medium such as a porous metal medium comprising metal fibers, the free area surface S is substantially completely coated with the coating layer. This means that the free area surface S is coated over the whole thickness of the medium.
With "substantially completely" is meant that although there may be some accidental uncoated spots there are no structural uncoated areas.
All the porous media according to the present invention showed that at least 95 % of the total free area surface S was coated.
For most embodiments more than 99 % of the total free area surface S was coated.

A second characteristic of the coating layer according to the present invention is that the coating is conformal.
With a conformal coating is meant a coating that is conserving the shape of the non-coated porous medium. A conformal coating is thus exactly or almost exactly replicating the shape of the surface of the non-coated porous medium.
With "substantially conformal" is meant that although there may be some small, accidental deviations over the surface and over the thickness of the medium, there are no structural deviations, neither over the surface of the medium, nor over the thickness of the medium.

A third characteristic of a coating layer according to the present invention is that the coating layer has a substantially uniform composition over the whole free area surface.

With "a substantially uniform composition" is meant that although there may be some small, accidental deviations in composition over the surface and over the thickness of the medium, there are no structural deviations neither over the surface of the medium nor over the thickness of the medium.

A further characteristic of a coating layer according to the present invention is that the coating layer has substantially the same thickness over the whole free area surface.
With "substantially the same thickness" is meant that although there can be some small deviations in the thickness over the surface of the medium and over the thickness of the medium, there are no structural deviations neither over the surface of the medium nor over the thickness of the medium.
For a coating thickness of 10 nm, deviations in thickness are at the most 1 nm; for a coating thickness of 100 nm, deviations in thickness are at the most 10 nm and for a coating thickness of 1000 nm, deviations in thickness are at the most 100 nm.

### Coating layer

In principle any composition of coating layers can be considered. Preferred coating layers comprise oxides, nitrides, fluorides and metals.
As oxides Al₂O₃, TiO₂, SiO₂, ZrO₂, HfO₂, Ta₂O₅, Nb₂O₅, Y₂O₃, MgO, CeO₂, La₂O₃, SrTiO₃, BaTiO₃, In₂O₃, SnO₂, ZnO, Ga₂O₃, NiO, YBa₂Cu₃O₇₋ₓ, LaCoO₃, LaNiO can be considered.
Examples of nitrides comprise AIN, GaN, InN, SiNx, TiN, TaN, Ta₃N₅, NbN and MoN.
Examples of fluorides comprise CaF₂, SrF₂ and ZnF₂.
Examples of metals comprise Si, Ge, Cu, Mo, Ti, W, Ni, Ag, Au, Pt and Pd.

The coating layer has preferably a stoechiometric composition.

### Thickness of coating layer

In principle, any thickness of the coating layer can be obtained as the thickness of the coating layer can be controlled perfectly at an atomic scale by the deposition technique of ALD.
However, the thickness of the coating layer is preferably between 10 and 1000 nm and more preferably between 50 and 500 nm, as for example 100 or 200 nm.

A great advantage of the present invention is that coating layers having a minimal thickness can be obtained.
A further advantage of the invention is that even thin coating layers such as coating layers having a thickness lower than 50 nm such as 20 nm are closed layers.

According to a second aspect of the present invention the use of a coated porous metal medium as described before as filter medium is provided.
Depending on the coating type of the coated porous metal medium, the filter medium can be used for filtration at high temperature, for filtration of corrosive fluids or for aggressive chemicals.

The coating layer applied on the free area surface S of the porous medium is so thin that the filter characteristics of the non-coated medium such as the mean pore size, the porosity and the filter rating are maintained by applying the coating layer.

According to a third aspect of the present invention a method to manufacture a coated porous metal medium comprising metal particles is provided.
The method comprises the steps of
- providing a porous metal medium comprising metal particles, said metal particles defining a free area surface S;
   applying a coating layer by atomic layer deposition on said free area surface S in such a way that said coating layer is covering said free area surface S substantially completely, said coating layer being substantially conformal, being substantial uniform in composition and having substantially the same thickness over the whole free area surface.

### Description of the preferred embodiments of the invention.

In an embodiment of the present invention, a non-woven porous metal medium comprising stainless steel fibers (316L) having a diameter of 2 µm is coated by means of atomic layer deposition (ALD).
The uncoated non-woven porous metal medium has a porosity of 86 %, a thickness of 500 µm.
The stainless steel fibers define a free area surface S of 150 m²/m² macroscopic surface of the non-woven porous metal medium.
Using ALD, the medium was conformally coated with a stoichiometric Al₂O₃ coating layer. The Al₂O₃ coating layer has a thickness of 80 nm.

After the application of the coating layer, the porosity of the coated medium remains the same as the porosity of the uncoated medium, i.e. 86%.

By means of SEM, it was verified that the free area surface S is completely coated with the coating layer, i.e. that all steel fibers are covered by the Al₂O₃ coating layer.

The coated porous metal medium described above is compared to an uncoated porous metal medium in an electrochemical corrosion analysis. The corrosion current is measured in an electrolyte. The used electrolyte comprises 0.1 N H₂SO₄ in 90 % ethanol. This type of electrolyte is chosen in order to achieve an optimal wettability (contact angle of 0°) so that the corrosion behavior of the free area surface S of the porous medium can be measured.

The obtained corrosion current for the uncoated and the coated porous metal medium, expressed as µA/cm² of macroscopic porous medium is given in Table 1.

**Table 1**

| Sample | Corrosion current (0.1 N H₂SO₄ in 90 % ethanol) (µA/cm²) |
|---|---|
| Uncoated porous metal medium | 6.02 |
| Coated porous metal medium | 0.23 |

The data of Table 1 show that the resistance of the coated porous metal medium is more than 96 % higher than the resistance of the uncoated porous metal medium.
Because the wettability of used electrolyte is considered to be 100 %, from the date of Table 1, it can be concluded that the total free area surface S of the porous metal medium is substantially completely coated as the coverage is more than 96 % of the total free area surface.

To further demonstrate the difference between a coated porous metal medium according to the present invention and an uncoated porous metal medium, the above mentioned coated and uncoated porous metal medium are subjected to a heat treatment (500 °C during 12 hours).
The weight of the media were determined before and after the heat treatment.
After the heat treatment the weight of the uncoated porous metal medium was increased with 1.4 % whereas the weight of the coated porous metal medium according to the present invention showed only a small increase of 0.1 %.

The above mentioned tests are thus illustrating that by using ALD, a substantially uniform and conformal thin coating layer can be deposited resulting in a greatly improved corrosion resistance.
As mentioned above, depending on the type of the coating layer that is deposited on the porous metal medium different functionalities can be given to the medium.

## Claims

1. A porous metal medium comprising metal particles, said metal particles defining a free area surface S; said free area surface S being substantially completely coated with a coating layer, said coating layer being substantially conformal, being substantially uniform in composition and having substantially the same thickness over the whole free area surface.

2. A porous metal medium according to claim 1, whereby said metal particles comprise metal powder and/or metal fibers.

3. A porous metal medium according to claim 1 or 2, whereby said metal particles comprise steel particles such as stainless steel particles.

4. A porous metal medium according to claim 2 or 3, whereby said metal fibers have a diameter ranging between 1 and 100 µm.

5. A porous metal medium according to any one of the preceding claims, whereby said porous metal medium comprises a non-woven porous metal medium comprising sintered metal fibers.

6. A porous metal medium according to any one of claims 1 to 4, whereby said porous metal medium comprises sintered metal powder.

7. A porous metal medium according to any one of the preceding claims, whereby said coating layer is applied by atomic layer deposition.

8. A porous metal medium according to any one of the preceding claims, whereby said coating layer comprises an oxide, a nitride, a fluoride or a metal.

9. A porous metal medium according to claim 8, whereby said oxide is selected from the group consisting of Al₂O₃, TiO₂, SiO₂, ZrO₂, HfO₂, Ta₂O₅, Nb₂O₅, Y₂O₃, MgO, CeO₂, La₂O₃, SrTiO₃, BaTiO₃, In₂O₃, SnO₂, ZnO, Ga₂O₃, NiO, YBa₂Cu₃O₇₋ₓ, LaCoO₃, ad LaNiO.

10. A porous metal medium according to any one of the preceding claims, whereby the composition of said coating layer is stoechiometric.

11. A porous metal medium according to any one of the preceding claims, whereby the thickness of said coating layer is ranging between 10 and 1000 nm.

12. Use of a porous metal medium as defined in any one of claims 1 to 11 as filter medium.

13. A method to manufacture a porous metal medium, said method comprising the steps of
- providing a porous metal medium comprising metal particles, said metal particles defining a free area surface S;
- applying a coating layer on said free surface area S by atomic layer deposition, said coating layer covering said free area surface S substantially completely and said coating layer being substantially conformal and substantially uniform in composition and in thickness over said free area surface.

## Patentansprüche

1. Poröses Metallmedium, das Metallteilchen umfasst, wobei die Metallteilchen eine freie Oberfläche S definieren; wobei die freie Oberfläche S weitgehend vollständig mit einer Beschichtungsschicht beschichtet ist, wobei die Beschichtungsschicht weitgehend konformal ist, eine weitgehend einheitliche Zusammensetzung aufweist und über die gesamte freie Oberfläche weitgehend die gleiche Dicke aufweist.

2. Poröses Metallmedium nach Anspruch 1, wobei die Metallteilchen Metallpulver und/oder Metallfasern umfassen.

3. Poröses Metallmedium nach Anspruch 1 oder 2, wobei die Metallteilchen Stahlteilchen wie Edelstahlteilchen umfassen.

4. Poröses Metallmedium nach Anspruch 2 oder 3, wobei die Metallfasern einen Durchmesser im Bereich zwischen 1 und 100 µm aufweisen.

5. Poröses Metallmedium nach einem der vorhergehenden Ansprüche, wobei das poröse Metallmedium ein nicht gewebtes poröses Metallmedium umfasst, welches Sintermetallfasern umfasst.

6. Poröses Metallmedium nach einem der Ansprüche 1 bis 4, bei dem das poröse Metallmedium Sintermetallpulver umfasst.

7. Poröses Metallmedium nach einem der vorhergehenden Ansprüche, wobei die Beschichtungsschicht durch Atomlagenabscheidung aufgebracht wird.

8. Poröses Metallmedium nach einem der vorhergehenden Ansprüche, wobei die Beschichtungsschicht ein Oxid, ein Nitrid, ein Fluorid oder ein Metall umfasst.

9. Poröses Metallmedium nach Anspruch 8, wobei das Oxid aus der Gruppe bestehend aus Al₂O₃, TiO₂, SiO₂, ZrO₂, HfO₂, Ta₂O₅, Nb₂O₅, Y₂O₃, MgO, CeO₂, La₂O₃, SrTiO₃, BaTiO₃, In₂O₃, SnO₂, ZnO, Ga₂O₃, NiO, YBa₂Cu₃O₇₋ₓ, LaCoO₃ und LaNiO ausgewählt ist.

10. Poröses Metallmedium nach einem der vorhergehenden Ansprüche, wobei die Zusammensetzung der Beschichtungsschicht stöchiometrisch ist.

11. Poröses Metallmedium nach einem der vorhergehenden Ansprüche, wobei die Dicke der Beschichtungsschicht im Bereich zwischen 10 und 1000 nm liegt.

12. Verwendung eines porösen Metallmediums gemäß einem der Ansprüche 1 bis 11 als Filtermedium.

13. Verfahren zur Herstellung eines porösen Metallmediums, das die folgenden Schritte umfasst:
- Bereitstellen eines porösen Metallmediums, das Metallteilchen umfasst, wobei die Metallteilchen eine freie Oberfläche S definieren;
- Aufbringen einer Beschichtungsschicht auf die freie Oberfläche S durch Atomlagenabscheidung, wobei die Beschichtungsschicht weitgehend die freie Oberfläche S bedeckt und die Beschichtungsschicht weitgehend konformal ist und eine weitgehend einheitliche Zusammensetzung aufweist und über die freie Oberfläche eine einheitliche Dicke aufweist.

## Revendications

1. Couche métallique poreuse comprenant des particules métalliques, lesdites particules métalliques définissant une surface libre S ; ladite surface libre S étant presque entièrement recouverte d'une couche de revêtement, ladite couche de revêtement étant sensiblement conforme, étant sensiblement uniforme en composition et ayant sensiblement la même épaisseur sur la totalité de la surface libre.

2. Couche métallique poreuse selon la revendication 1, lesdites particules métalliques comprenant une poudre métallique et/ou des fibres métalliques.

3. Couche métallique poreuse selon la revendication 1 ou 2, lesdites particules métalliques comprenant des particules d'acier telles que des particules d'acier inoxydable.

4. Couche métallique poreuse selon la revendication 2 ou 3, lesdites fibres métalliques ayant un diamètre variant entre 1 et 100 µm.

5. Couche métallique poreuse selon l'une quelconque des revendications précédentes, ladite couche métallique poreuse comprenant une couche métallique poreuse non tissée comprenant des fibres métalliques frittées.

6. Couche métallique poreuse selon l'une quelconque des revendications 1 à 4, ladite couche métallique poreuse comprenant une poudre métallique frittée.

7. Couche métallique poreuse selon l'une quelconque des revendications précédentes, ladite couche de revêtement étant appliquée par dépôt de couches atomiques.

8. Couche métallique poreuse selon l'une quelconque des revendications précédentes, ladite couche de revêtement comprenant un oxyde, un nitrure, un fluorure ou un métal.

9. Couche métallique poreuse selon la revendication 8, ledit oxyde étant choisi dans le groupe constitué par Al₂O₃, TiO₂, SiO₂, ZrO₂, HfO₂, Ta₂O₅, Nb₂O₅, Y₂O₃, MgO, CeO₂, La₂O₃, SrTiO₃, BaTiO₃, In₂O₃, SnO₂, ZnO, Ga₂O₃, NiO, YBa₂Cu₃O₇₋ₓ, LaCoO₃ et LaNiO.

10. Couche métallique poreuse selon l'une quelconque des revendications précédentes, la composition de ladite couche de revêtement étant stoechiométrique.

11. Couche métallique poreuse selon l'une quelconque des revendications précédentes, l'épaisseur de ladite couche de revêtement variant entre 10 et 1000 nm.

12. Utilisation d'une couche métallique poreuse telle que définie dans l'une quelconque des revendications 1 à 11 comme couche filtrante.

13. Procédé de fabrication d'une couche métallique poreuse, ledit procédé comprenant les étapes consistant à
- se procurer une couche métallique poreuse comprenant des particules métalliques, lesdites particules métalliques définissant une surface libre S ;
- appliquer une couche de revêtement sur ladite surface libre S par dépôt de couches atomiques, ladite couche de revêtement recouvrant presque entièrement ladite surface libre S et ladite couche de revêtement étant sensiblement conforme et sensiblement uniforme en composition et en épaisseur sur ladite surface libre.
